

July 5, 1960

H. A. AMBROSE

2,943,925

RESIDUAL FUEL OILS

Filed Aug. 27, 1956



INVENTOR.  
BY HENRY A. AMBROSE

*Herbert Blaauw*  
HIS ATTORNEY

1

2,943,925

## RESIDUAL FUEL OILS

Henry A. Ambrose, Penn Township, Allegheny County, Pa., assignor to Gulf Research & Development Company, Pittsburgh, Pa., a corporation of Delaware

Filed Aug. 27, 1956, Ser. No. 606,413

9 Claims. (Cl. 44—66)

This invention relates to vanadium-containing petroleum fuels. More particularly, it is concerned with rendering non-corrosive those residual fuels which contain such an amount of vanadium as normally to yield a corrosive vanadium-containing ash upon combustion.

This application is a continuation-in-part of my prior copending application Serial No. 227,108, filed May 18, 1951.

It has been observed that when a residual type fuel oil containing substantial amounts of vanadium is burned in furnaces, boilers and gas turbines, the ash resulting from combustion of the fuel oil is highly corrosive to materials of construction at elevated temperatures and attacks such parts as boiler tubes, hangers, turbine blades, and the like. These effects are particularly noticeable in gas turbines. Large gas turbines show promise of becoming an important type of industrial prime mover. However, economic considerations based on the efficiency of the gas turbine dictate the use of a fuel for this purpose which is cheaper than a distillate diesel fuel; otherwise, other forms of power such as diesel engines become competitive with gas turbines.

One of the main problems arising in the use of residual fuel oils in gas turbines is the corrosiveness induced by those residual fuels containing sufficient amounts of vanadium to cause corrosion problems. Where no vanadium is present or the amount of vanadium is small, no appreciable corrosion is encountered. While many residual fuel oils as normally obtained in the refinery contain so little vanadium, or none, as to present no corrosion problems, such non-corrosive fuel oils are not always available at the point where the oil is to be used. In such instance, the cost of transportation of the non-corrosive oil to the point of use is often prohibitive, and the residual oil loses its competitive advantage. These factors appear to militate against the extensive use of residual fuel oils for gas turbines. Aside from corrosion, the formation of deposits upon the burning of a residual fuel in a gas turbine may result in unbalance of the turbine blades, clogging of openings and reducing thermal efficiency of the turbine.

Substantially identical problems are encountered when using a solid residual petroleum fuel containing substantial amounts of vanadium. These fuels are petroleum residues obtained by known methods of petroleum refining such as deep vacuum reduction of asphaltic crudes to obtain solid residues, visbreaking of liquid distillation bottoms followed by distillation to obtain solid residues, coking of liquid distillation bottoms, and the like. The solid residues thus obtained are known variously as petroleum pitches or cokes and find use as fuels. Since the vanadium content of the original crude oil tends to concentrate in the residual fractions, and since the processing of the residual fractions to solid residues results in further concentration of the vanadium in the solid residues, the vanadium corrosion problem tends to be intensified in using the solid residues as fuel.

The vanadium-containing ash present in the hot flue

2

gas obtained from the burning of a residual fuel containing substantial amounts of vanadium compounds causes "catastrophic" corrosion of the turbine blades and other metal parts in a gas turbine. The corrosive nature of the ash appears to be due to its vanadium oxide content. Certain inorganic compounds of vanadium, such as vanadium oxide ( $V_2O_5$ ), which are formed on combustion of a residual fuel oil containing vanadium compounds, vigorously attack various metals, their alloys, and other materials at the elevated temperatures encountered in the combustion gases, the rate of attack becoming progressively more severe as the temperature is increased. The vanadium-containing ash forms deposits on the parts affected and corrosively reacts with them. It is a hard, adherent material when cooled to ordinary temperatures.

It is to be noted that the corrosion of materials at high temperatures by the hot ash resulting from the combustion of a vanadium-containing residual fuel is to be distinguished from the type of corrosion occurring at atmospheric or slightly elevated temperatures, generally in the presence of air and moisture. Under the latter conditions, an ash containing vanadium oxide has no significant corrosive effect. The corrosion problem described herein may therefore properly be termed a problem of "hot corrosion."

The economic factors involved preclude any extensive treatment of vanadium-containing residual fuels to remove the vanadium therefrom or to mitigate its effects. The vanadium compounds in residual oils are not removed by centrifuging or by the conventional chemical refining treatments.

In my prior copending application Serial No. 227,108, previously referred to, I have shown that oil-soluble and oil-dispersible metal salts of an acidic organic compound, the metal of said metal salts, being selected from the group consisting of the metals of Groups I, II, III, IV, VI, VII and VIII of the Periodic Table of Mendeleef, can be employed in minor amounts in a residual fuel oil yielding a corrosive vanadium-containing ash upon combustion to retard the corrosiveness of the ash.

I have now discovered that not all of the metal salts of my copending application are of equal effectiveness and that manganese salts of an acidic organic compound show outstanding superiority in retarding, and in fact, substantially preventing corrosion. The present invention therefore relates to residual petroleum fuels containing vanadium in an amount sufficient to yield a corrosive vanadium-containing ash upon combustion, and containing, in a minor amount sufficient to retard the corrosiveness of the ash, an oil-soluble or oil-dispersible manganese salt of an acidic organic compound.

The single figure of the drawing shows an apparatus for testing the corrosiveness of residual fuel oil compositions.

The type of residual fuel oils to which my invention is directed is exemplified by No. 5, No. 6 and Bunker "C" fuel oils which contain a sufficient amount of vanadium to form a corrosive ash upon combustion. These are residual type fuel oils obtained from petroleum by methods known to the art. For example, residual fuel oils are obtained as liquid residua by the conventional distillation of total crudes, by atmospheric and vacuum reduction of total crudes, by the thermal cracking of topped crudes, by visbreaking heavy petroleum residua, and other conventional treatments of heavy petroleum oils. Residua thus obtained are sometimes diluted with distillate fuel oil stocks, known as "cutter" stocks, and the invention also includes residual fuel oils so obtained, provided that such oils contain sufficient vanadium normally to exhibit the corrosion characteristics described herein. It should be understood that distillate fuel oils themselves contain either no vanadium or such small amounts as

to present no problem of hot corrosion. The total ash from commercial residual fuel oils usually ranges from about 0.02 to 0.2 percent by weight. The vanadium pentoxide ( $V_2O_5$ ) content of such ashes ranges from zero to trace amounts up to about 5 percent by weight for low vanadium stocks, exhibiting no significant vanadium corrosion problem, to as much as 85 percent by weight for some of the high vanadium stocks, exhibiting severe corrosion.

The type of vanadium-containing solid residual fuels to which the invention is directed is exemplified by the coke obtained in known manner by the delayed thermal coking or fluidized coking of topped or reduced crude oils and by the pitches obtained in known manner by the deep vacuum reduction of asphaltic crudes to obtain solid residues. These materials have ash contents of the order of 0.18 percent by weight, more or less, and contain corrosive amounts of vanadium when prepared from stocks containing substantial amounts of vanadium. A typical pitch exhibiting corrosive characteristics upon combustion had a softening point of 347° F. and a vanadium content, as vanadium, of 578 parts per million.

As disclosed in my prior copending application, the manganese salts of the invention can be prepared from any acidic organic compound that forms oil-soluble or oil-dispersible metal compounds. Representative examples of the salts of the invention include oil-soluble and oil-dispersible manganese salts of (1) the fatty acids of at least 5 carbon atoms, e.g., valeric, caproic, 2-ethyl-hexanonic, oleic, palmitic, stearic, linoleic, tall oil, and the like; (2) oil-soluble alkylaryl sulfonic acids, e.g., oil-soluble petroleum sulfonic acids and dodecylbenzenesulfonic acid; (3) long chain alkylsulfuric acids, e.g., lauryl sulfuric acid; (4) petroleum naphthenic acids; (5) rosin and hydrogenated rosin; (6) alkyl phenols, e.g., iso-octyl phenol, t-butylphenol and the like; (7) alkylphenol sulfides, e.g., bis(iso-octyl phenol)monosulfide, bis(t-butylphenol) disulfide, and the like; and (8) oil-soluble phenolformaldehyde resins, e.g., the Amberols, such as t-butylphenol-formaldehyde resin, and the like. Since the salts or soaps of such acidic organic compounds as the fatty acids, naphthenic acids and rosins are readily available or can easily be prepared, these are preferred materials. Particularly preferred are manganese naphthenate, manganese oleate, manganese tallate (tall oil soaps) and manganese rosinate.

The requirement for oil-solubility or dispersibility of the manganese salts of the invention is to insure uniform blending thereof when employed with a residual fuel oil. It would obviously be undesirable for the bulk of the additive to be concentrated in a small portion of the fuel oil while the remainder of the oil contained little or no additive. The requirement for uniform blending of the manganese salts is therefore satisfied by the use of oil-soluble or oil-dispersible compounds. As will be apparent to those skilled in the art, the distinction between oil-solubility and oil-dispersibility is a matter of degree, it being sufficient for present purposes that a fairly stable dispersion of the dispersible additives be obtained, or that redispersion of a settled additive can be easily accomplished by simple agitation.

With the solid residual fuels, incorporation of the oil-soluble or oil-dispersible manganese salts is accomplished in several ways. The salts can be suspended or dissolved in the liquid vanadium-containing residual stocks or crude oil stocks from which the solid residual fuels of the invention are derived, and the mixture can then be subjected to the refining process which will produce the solid fuel. For example, in the production of a pitch by the deep vacuum reduction of an asphaltic crude oil, manganese naphthenate is slurried with the oil in proportion to the vanadium content thereof, and the whole subjected to deep vacuum reduction to obtain a pitch containing uniformly dispersed therein the manganese naph-

thenate. Alternatively, particles of the solid residual fuels in question can be coated or impregnated with a concentrated naphtha solution of the manganese salt in the proportion required in relation to the vanadium content, and the aggregate then dried to obtain solid fuel particles impregnated with the additive. As still another alternative, particularly with a pitch which is withdrawn in molten form from the processing vessel, the additive can be mixed with the molten pitch and the mixture allowed to solidify after which it is ground to the desired size. Of course, in the case of either liquid or solid residual fuels, the additive can be separately fed into the burner as a concentrated solution, preferably in admixture with the fuel.

As has been stated, the manganese salts are employed in a small amount with respect to the vanadium-containing residual fuel, sufficient to retard the corrosiveness of the ash. Ordinarily, to achieve practical corrosion retardation, it is desirable to employ such an amount of additive as to result in at least about 3 atom weights of the manganese of the salt per atom weight of the vanadium in the fuel oil. Preferably, the atom weight ratio, Mn:V, is 6:1, although larger amounts of the salts can be employed. Since on a weight basis in relation to the fuel the amounts of additive are small, it is desirable to make concentrated solutions or dispersions of the additive in a naphtha, kerosene or gas oil for convenience of compounding.

The following specific examples are further illustrative of my invention.

#### Example 1

In a 50 gram portion of a No. 6 residual fuel oil having an ash content of 0.055 percent by weight and a vanadium content of 0.015 percent by weight, there is dispersed 0.5 percent by weight of manganese naphthenate. The atom ratio of manganese to vanadium in the dispersion is 2:1.

#### Example 2

With a residual fuel oil having an ash content of 0.037 percent by weight and containing 166 parts per million of vanadium, uniformly blend 0.9 percent by weight of a 6 percent concentrate of manganese naphthenate in naphtha. This yields an atom ratio, Mn:V, of about 3:1.

#### Example 3

To the same residual fuel oil of Example 2, add 1.8 percent by weight of the same concentrate of manganese naphthenate in naphtha. This yields a Mn:V atom ratio of about 6:1.

#### Example 4

A fuel oil composition according to the invention is prepared by blending 2.23 percent by weight of a concentrate in naphtha of manganese linoleate (Mn content 4.35 percent) with a residual fuel oil having an ash content of 0.04 percent by weight and a vanadium content of 180 parts per million. An atom ratio, Mn:V, of 5:1 is obtained.

#### Example 5

Another composition according to the invention is prepared by blending manganese tallate in a vanadium-containing residual fuel oil to obtain a Mn:V atom ratio of 4.5:1.

#### Example 6

Melt a solid petroleum pitch obtained from the deep vacuum reduction of an asphaltic crude. This pitch has a softening point of 347° F. and a vanadium content of 578 parts per million. While the pitch is in molten form add and uniformly blend therein 3.1 percent by weight of the manganese naphthenate concentrate of Example 2. Upon cooling and solidification, grind the mixture to about 150 mesh. The resulting fuel has an atom ratio, Mn:V, of about 3:1.

Similar compositions are prepared using manganese

octoate (2-ethylhexanoate), stearate, octylphenolate, as well as the other acidic organic compounds disclosed herein.

In order to demonstrate the effectiveness of the manganese salts of the invention, the composition of Example 1 is placed in a 4" diameter 18-8 stainless steel dish and the dish is heated until the fire temperature of the oil is reached and the oil ignites. After the oil has burned itself out, the dish containing the residue from the ignition is placed in a muffle furnace and heated for 8 hours at 1350° F. At the end of this time, the dish is allowed to cool slowly and the nature of the ash is determined by inspection. An identical residual fuel oil without the manganese naphthenate is run for purposes of comparison. The results obtained are:

| Additive              | Nature of Ash                             |
|-----------------------|-------------------------------------------|
| None                  | Hard and firmly adhered to walls of dish. |
| Manganese Naphthenate | Loose, powdery, non-adherent residue.     |

In order to test the effectiveness of the additives of this invention under conditions of burning residual fuels in a gas turbine, the apparatus shown in the drawing is employed. As shown in the drawing, the residual oil water tests is introduced through line 10 into a heating coil 11 disposed in a tank of water 12 maintained at such temperature that the incoming fuel is preheated to a temperature of approximately 212° F. From the heating coil 11 the preheated oil is passed into an atomizing head designated generally as 13. The preheated oil passes through a passageway 14 into a nozzle 15 which consists of a #26 hypodermic needle of approximately 0.008 inch I.D. and 0.018 inch O.D. The tip of the nozzle is ground square and allowed to project slightly through an orifice 16 of approximately 0.020 inch diameter. The orifice is supplied with 65 p.s.i.g. air for atomization of the fuel into the combustion chamber 21. The air is introduced through line 17, preheat coil 18 in tank 12, and air passageways 19 and 20 in the atomizing head 13. The combustion chamber 21 is made up of two concentric cylinders 22 and 23, respectively, welded to two end plates 24 and 25. Cylinder 22 has a diameter of 2 inches and cylinder 23 has a diameter of 3 inches; the length of the cylinders between the end plates is 8½ inches. End plate 24 has a central opening 26 into which the atomizing head is inserted. End plate 25 has a one (1) inch opening 27 covered by a baffle plate 28 mounted in front of it to prevent direct blast of flame on the test specimen 29. Opening 27 in end plate 25 discharges into a smaller cylinder 30 having a diameter of 1½ inches and a length of 6 inches. The specimen 29 is mounted near the downstream end of the cylinder approximately 1¾ inches from the outlet thereof. Combustion air is introduced by means of air inlet 31 into the annulus between cylinders 22 and 23, thereby preheating the combustion air, and then through three pairs of ¾ inch tangential air inlets 32 in the inner cylinder 22. The first pair of air inlets are spaced ¼ inch from end plate 24; the second pair ¾ inch from the first; and the third 3 inches from the second. The additional heating required to bring the combustion products to test temperature is supplied by an electric heating coil 33 surrounding the outer cylinder 23. The entire combustion assembly is surrounded by suitable insulation 34. The test specimen 29 is a metal disc one inch in diameter by 0.125 inch thick, with a hole in the center by means of which the specimen is attached to a tube 35 containing thermocouples. The specimen and tube assembly are mounted on a suitable stand 36.

In conducting a test in the above-described apparatus, a weighted metal specimen is exposed to the combustion products of a residual fuel oil, the specimen being main-

tained at a selected test temperature of 1350°, 1450° or 1550° F. by the heat of the combustion products. The test is usually run for a period of 100 hours with the rate of fuel feed being ½ pound per hour and the rate of atomizing air feed being 2 pounds per hour. The combustion air entering through air inlet 31 is fed at 25 pounds per hour. At the end of the test run the specimen is reweighed to determine the weight of deposits and is then descaled with a conventional alkaline descaling salt 10 in molten condition at 475° C. After descaling, the specimen is dipped in 6 N hydrochloric acid containing a conventional pickling inhibitor, and is then washed, dried and weighed. The loss in weight of the specimen after descaling is the corrosion loss.

15 A test is conducted in the apparatus just described using a 25-20 stainless steel as the test specimen. The test is run for 100 hours at a temperature of 1450° F. under the conditions described above. The oil employed is a residual fuel oil having an ash content of 0.037 percent and 20 containing 166 parts per million of vanadium. Comparative tests are run with the oil containing no additive and with the compositions of Examples 2 and 3.

| 25                                 | Corrosion, Wt. Loss, Mg./Sq. in. | Deposits    |                     |
|------------------------------------|----------------------------------|-------------|---------------------|
|                                    |                                  | Mg./Sq. in. | Texture             |
| Fuel Oil Alone                     | 992                              | 319         | Hard, crusty scale. |
| Fuel Oil With Additive (Example 2) | 92                               | 144         | Black powder.       |
| Fuel Oil With Additive (Example 3) | 4                                | 43          | Light, powdery ash. |

In order to demonstrate the superior effectiveness of the manganese additives of the invention, comparative tests are run under identical conditions in the apparatus described herein with corrosive vanadium-containing residual oils containing manganese naphthenate, calcium naphthenate and oil-soluble barium petroleum sulfonate as corrosion retarding additives. The test specimens are 25-20 stainless steel, and as described above, the test is run for 100 hours at a temperature of 1450° F. Each additive, i.e., the manganese naphthenate, calcium naphthenate and barium petroleum sulfonate, is employed in an amount sufficient to give an identical atom weight ratio of metal to the vanadium of 6:1. The results obtained are shown in the following table:

| 50                                         | Corrosion, Wt. Loss, Mg./Sq.in. | Deposits    |                     |
|--------------------------------------------|---------------------------------|-------------|---------------------|
|                                            |                                 | Mg./Sq. in. | Texture             |
| No. 6 Fuel Oil With Manganese Naphthenate. | 4                               | 43          | Light, powdery ash. |
| No. 6 Fuel Oil With Calcium Naphthenate.   | 81                              | 226         | Powdery deposit.    |
| No. 6 Fuel Oil With Barium Sulfonate.      | 170                             | 178         | Light scale.        |

The above results clearly show the superiority of the manganese salts of the invention to other corrosion retarding additives. Corrosion has been reduced to a negligible amount, and deposit formation has been minimized.

Typical analyses of the stainless steels employed in the above description are shown in the following table in percent by weight:

| 70  |         | 18-8    | 25-20 |
|-----|---------|---------|-------|
|     |         | Cr.     | Ni.   |
| Cr. | 18.91   | 25      |       |
| Ni. | 8.62    | 20      |       |
| C.  | 0.12    | 0.08    |       |
| Mn. | 0.62    | 2.0     |       |
| Si. | 0.60    | 1.5     |       |
| S.  |         | 0.03    |       |
| P.  |         | 0.04    |       |
| Fe. | Balance | Balance |       |

The above examples clearly demonstrate the effectiveness of the manganese additives of the invention in reducing the corrosivity of vanadium-containing residual fuels, and also in reducing the amount of ash deposits obtained. Furthermore, the character of the deposits has been radically changed from a hard, adherent scale to a light, soft and powdery material which is more readily blown out by the combustion draft in a turbine, furnace or boiler and which can more easily be removed from the affected parts.

Resort may be had to such modifications and variations as fall within the spirit of the invention and the scope of the appended claims.

I claim:

1. A fuel composition comprising a major amount of a residual petroleum fuel yielding a corrosive vanadium-containing ash upon combustion, and a small amount of a salt selected from the class consisting of oil-soluble and oil-dispersible manganese salts of an acidic organic compound sufficient to retard the corrosiveness of said ash.

2. The composition of claim 1, wherein the manganese salt is employed in an amount sufficient to yield at least about 3 atom weights of manganese per atom weight of vanadium.

3. The composition of claim 1, wherein the fuel is a solid residual petroleum fuel.

4. The composition of claim 1, wherein the acidic organic compound is selected from the class consisting of fatty acids of at least 5 carbon atoms, naphthenic acids and rosins.

5. A fuel composition comprising a major amount of a residual petroleum fuel oil yielding a corrosive vanadium-containing ash upon combustion and an amount of a manganese salt sufficient to yield from about 3 to about 6 atom weights of manganese per atom weight of vanadium in said oil, said salt being selected from the class consisting of oil-soluble and oil-dispersible manganese salts of fatty acids of at least 5 carbon atoms, naphthenic acids and rosins.

10 6. The composition of claim 5, wherein the manganese salt is manganese naphthenate.

7. The composition of claim 5, wherein the manganese salt is manganese tallate.

8. The composition of claim 5, wherein the manganese salt is manganese rosinate.

20 9. The composition of claim 5, wherein the manganese salt is manganese linoleate.

References Cited in the file of this patent

UNITED STATES PATENTS

2,230,642 Fischer et al. Feb. 4, 1941

UNITED STATES PATENT OFFICE  
CERTIFICATE OF CORRECTION

Patent No. 2,943,925

July 5, 1960

Henry A. Ambrose

It is hereby certified that error appears in the printed specification of the above numbered patent requiring correction and that the said Letters Patent should read as corrected below.

Column 3, line 38, for "(t-tbutylphenol)" read -- (t-butyphenol) --; column 5, line 14, for "in" read -- is --; line 27, for "water" read -- under --.

Signed and sealed this 20th day of December 1960.

(SEAL)

Attest:

KARL H. AXLINE  
Attesting Officer

ROBERT C. WATSON  
Commissioner of Patents